

J. I. SOUTHER.

TREATMENT OF FLUE DUST.

APPLICATION FILED MAY 15, 1905.

1,041,363.

Patented Oct. 15, 1912.



WITNESSES.

Elmer Leavay  
Charles M. Chambers.

INVENTOR.

John I. Souther:  
by Geo. E. Thackray  
his ATTORNEY.

# UNITED STATES PATENT OFFICE.

JOHN I. SOUTHER, OF WESTMONT, PENNSYLVANIA.

## TREATMENT OF FLUE-DUST.

1,041,363.

Specification of Letters Patent.

Patented Oct. 15, 1912.

Application filed May 15, 1905. Serial No. 260,462.

*To all whom it may concern:*

Be it known that I, JOHN I. SOUTHER, a citizen of the United States, residing in the borough of Westmont, in the county of Cambria and State of Pennsylvania, have invented certain new and useful Improvements in the Treatment of Flue-Dust; and I do hereby declare the following to be a full, clear, and exact description of the invention, such as will enable others skilled in the art to which it appertains to make and use the same.

In conducting metallurgical operations requiring the smelting or other treatment of ores and particularly those which contain a greater or less proportion of fine or pulverulent material and especially when using such ores in a blast or similar furnace, it is found that considerable percentages of said ores, consisting of the finer portions, are carried over from the smelting or other apparatus and deposited in the flues, dust-catchers, hot blast stoves or elsewhere, as may be readily understood. This deposit of fine ores is ordinarily called flue-dust, and in order to simplify the phraseology of this specification, I will confine my description herein to the flue-dust which accumulates in connection with the operation of a blast furnace smelting iron ore, although it will be understood that my treatment will apply equally well to flue-dust obtained from any other sources, or to fine ores of any kind or derivation. In order to simplify the language of the specification by using uniform expressions herein, I employ the term "flue-dust" as applying to any one of the finely divided materials which may be treated by my method, as will be readily understood by one skilled in this art. Under certain conditions, as heretofore explained, the amount of flue-dust which accumulates is very considerable, but if it is re-charged into the furnace in the attempt to smelt it, most of it is blown out again by the force of the blast, thus resulting in labor and expense without compensation.

My invention consists briefly in treating flue-dust by agglomerating or sintering it into rough lumpy form by means of high heat applied thereto, preferably in a revolving cylindrical furnace, using blast furnace gas as a fuel. In order to have this matter clearly understood, I have illustrated

on the accompanying sheet of drawings, one 55 form of apparatus which may be used for this purpose.

Referring to the accompanying sheet of drawings:—Figure 1 is a side elevation of a revolving cylinder showing the combustion chamber and stack in longitudinal section. Fig. 2 is a cross section taken on the line 2—2 of Fig. 1 and also showing a car in position to receive the material after it has received my treatment.

Referring now to the various characters of reference on the drawings:—1 represents a revoluble cylinder lined in its interior with refractory and preferably basic material, 2 indicates the driving mechanism for 60 revolving same by means of a motor (not shown), 3 is the combustion chamber in which the heating gases are brought into contact with the air and allowed to expand and reverberate for the purpose of obtaining a high heat in the lower end of the interior of the cylinder, and 4 is the draft stack.

5 represents a gas-main, 6 the gas burner or feeder-pipe connected therewith and 7 65 represents a gas-valve for regulating the supply of gas to the combustion chamber 3.

8 represents the finely divided flue-dust as it is being charged into the furnace cylinder, by means of the inclined chute as shown, 70 and 9 are lumps of flue-dust formed from the fine material as it is passed through the heated cylinder and becomes sintered or agglomerated into irregular hard lumps or masses.

10 is a delivery passage or chute formed in the rear portion of the combustion chamber for conveying the lumps to any convenient receptacle such as the car indicated at 11, and 12 represents a slide door or 75 damper for regulating the supply of gas to the combustion chamber.

In carrying out my treatment of flue-dust, it is charged into one end of the slowly revolving internally fired cylinder and as 80 it gradually travels toward the lower end thereof, it becomes heated more and more and thereby sintered or partially fused into irregular hard lumps or masses; this action being facilitated by the revolution of the 85 cylinder as may be understood. It will thus be seen that my treatment transforms the 90 finely divided material, which would be car-

ried away by the blast of a furnace, into solid lumps of substantial size, which can be charged into a furnace and smelted without loss, and although my treatment is a very simple and inexpensive one, therein resides a large part of its value.

I prefer to use waste gases from a blast furnace for heating the cylinder, as when burned in connection with a suitable supply 10 of air in a combustion chamber, as indicated on the drawing attached hereto, this waste gas will furnish a high degree of heat sufficient to accomplish the purpose intended, and as these gases are practically 15 waste products, the cost of fuel in connection with the operation is inconsiderable.

It will be noted that the finely divided flue-dust is charged into the upper end of the revolving and internally heated cylinder, 20 this end being the one nearest the stack and farthest removed from the fire, and on account of the length of the cylinder, the upper end is of a comparatively low temperature, which however, increases gradually 25 toward the lower or fire end, at which point it should preferably be white hot or of a temperature sufficient to sinter or clinker the material treated.

Although I do not limit myself to any 30 exact composition of flue-dust for my treatment, I can state that I have treated with success the flue-dust collected from an iron blast furnace which contains substantially the following ingredients, viz:—metallic 35 iron (contained in oxids) 57 per cent., silica and alumina 11 per cent., lime .2 per cent., coke and loss on ignition 8 per cent., sulfur, phosphorus and magnesia together, part of 1 per cent.

40 The temperature of fusion or agglomeration of fine ores or flue-dust is variable to a certain extent, depending upon the different characters of same and also varies with the different proportions of impurities which 45 they contain, such as sulfur, silica, alumina or silicates of alumina and other ingredients. In the conduct of my process, I therefore arrange the temperature in different parts of the furnace such that the upper 50 portion is comparatively cool, with gradually increasing temperature in said lower portion at the proper degree for partly fusing, agglomerating or sintering the particular kind of ore or flue-dust which I may be 55 treating at the time. It can be readily understood that a temperature which would cause one ore to fuse completely and melt would only partially fuse or sinter another ore and I therefore am careful to maintain 60 such a degree in the lower end of my apparatus that the material will be agglomerated

into masses or lumps, and not entirely melted or made liquid.

Having thus described my invention, what I claim and desire to secure by United States Letters Patent is:

1. The method of treating finely divided flue-dust which consists in charging the same into the upper end of an inclined revolving cylinder, heating the interior of said cylinder by means of blast furnace gas, the initial combustion of which is accomplished in a combustion chamber connected with the interior and lower end of said cylinder, whereby the combustion of said gas is partially perfected without said cylinder and near the lower end thereof, subjecting said flue-dust to gradually increasing temperature, as it travels toward the fire end of the cylinder, and thereby sintering or agglomerating the said flue-dust in masses or lumps, substantially as described.

2. The method of treating finely divided flue-dust or fine-ores which consists in charging the same into the upper end of an inclined revolving cylinder, heating the interior of said cylinder by means of a mixture of combustible gas and air, the initial combustion of which is accomplished in an expansive combustion chamber connected 90 with the lower end of the interior of said cylinder, whereby the combustion of said gases is partially perfected without said cylinder and the highest temperature attained near the lower end of the cylinder aforesaid, subjecting said flue-dust or fine-ores to gradually increasing temperature as they travel toward the fire end of the cylinder, and thereby sintering or agglomerating the same into masses or lumps by the combined 100 action of the gradually increasing temperature and rolling action.

3. The process of agglomerating fine-ores or residues, which consists in initially burning a mixture of combustible gas and air 105 out of the presence of said ores or residues and under such conditions that the resulting reaction-gases may expand and thoroughly mix and then passing the intensely hot products thereof over the ore or residue 110 to be agglomerated and progressively heating it to a temperature sufficient to partially fuse the impurities therein and cause them to become semi-plastic and sticky, and agitating the semi-plastic mass to cause 115 it to form into lumps.

In testimony whereof I hereto affix my signature in the presence of two witnesses.

JOHN I. SOUTHER.

Witnesses:

ELMER SEAVEY,  
CILAS. N. CHAMBERS.